

## UNITED STATES PATENT OFFICE

2,377,325

TREATMENT OF NONGELATIN  
EMULSIONS

John I. Crabtree and George T. Eaton, Rochester,  
N. Y., assignors to Eastman Kodak Company,  
Rochester, N. Y., a corporation of New Jersey  
No Drawing. Application October 16, 1942,

Serial No. 462,232

6 Claims. (Cl. 95—88)

This invention relates to improved photographic procedure for the treatment of non-gelatin photographic elements, and in particular to procedure for removing opalescence from photographic elements bearing a non-gelatin layer.

Various resin products which act as protective colloids or carriers have been proposed as a substitute for gelatin in photographic emulsions. Thus, resins such as cellulose nitrate, acetate, acetate-butylate; polyvinyl acetals such as polyvinyl acetaldehyde acetal and polyvinyl butyraldehyde acetal; cold water soluble polyvinyl acetaldehyde acetal; polyvinyl alcohol; and polyvinyl esters such as hydrolyzed vinyl acetate, have been used for this purpose. These substitutes are superior to gelatin in many respects, but it has been noted that with certain developing and fixing solutions or with certain forms of these gelatin substitutes a photographic element is obtained which is opalescent. The opalescence is apparently caused by the processing baths and is produced when the element comes in contact with the wash water. The element remains opalescent to a lesser degree when dry.

This invention has for its object to provide procedure for removing this opalescence. Another object is to provide procedure for removing the opalescence from processed non-gelatin emulsions. Other objects will appear hereafter.

These and other objects are accomplished by our invention which includes preventing or removing opalescence by treating the photographic element bearing a non-gelatin layer with a solution containing a member of the group consisting of ethylenediamines, ethanolamine, triethanolamine and alcohol.

In the following examples and description we have given several of the preferred embodiments of our invention, but it is to be understood that these are set forth for the purpose of illustration and not in limitation thereof.

It is preferred that the photographic element be treated with the substances mentioned immediately after processing, such as immediately after developing, fixing and/or washing. On the other hand much the same results can be obtained if the photographic element is maintained in a wet condition after the processing treatment and is treated to remove the opalescence at any subsequent time. It has been found that if the photographic element is first permitted to dry the opalescent quality is more difficult to remove. However, it is to be understood that our inven-

tion is applicable to the removal of opalescence from the non-gelatin emulsion at any stage in the processing treatment. If desired, the agents can be added to the washing bath or used in a supplemental bath just prior to washing.

We prefer to utilize the opalescent removing agents in aqueous solution in the following proportions:

|                    | Per cent solution |
|--------------------|-------------------|
| 10 Ethylenediamine | 1 to 60           |
| Ethanolamine       | 1 to 25           |
| Triethanolamine    | 1 to 20           |
| Alcohol            | 1 to 70           |

15 However, these proportions can be varied considerably and it is to be understood that our invention is not limited thereto. After treatment with the opalescent removing agent the photographic element is permitted to dry or is preferably first washed with water and then dried.

20 Our invention is applicable to the treatment of non-gelatin emulsions in general. However, it is of particular value in connection with the treatment of emulsions containing a cellulose ester carrier containing between about 26 and 33% acyl and of polyvinyl resins, particularly polyvinyl acetal resins.

## Example

30 A film carrying an emulsion of silver halide in a cellulose acetate-propionate carrier (22.5% acetyl and 17.0% propionyl) was exposed, developed, fixed and washed in the usual manner. When introduced into the washing bath the film became opalescent and remained so to a lesser degree when dried. The use of a supplemental bath immediately following fixing and containing 25% ethanolamine in aqueous solution resulted in a clear film on drying.

35 40 45 50 55 60 65 70 75 80 85 90 95 100

What we claim is:

1. The method of removing opalescence from a photographic element which comprises treating the opalescent photographic element bearing a non-gelatin layer containing a developed and fixed silver image with a solution of a member of the group consisting of ethylenediamine, ethanolamine, triethanolamine and alcohol.

2. The method of preventing or removing opalescence in a photographic element which comprises treating the photographic element bearing a non-gelatin layer containing a silver image with a solution containing a member of the group consisting of ethylenediamine, ethanolamine, triethanolamine and alcohol.

3. The method of preventing or removing opalescence in a photographic element which comprises treating the photographic element bearing a cellulose ester layer containing a developed and fixed silver image with a solution containing a member of the group consisting of ethylenediamine, ethanolamine, triethanolamine and alcohol.

4. The method of preventing or removing opalescence in a photographic element which comprises treating the photographic element bearing a cellulose ester layer having about 26-33% acyl content which layer contains a developed and fixed silver image with a solution containing a member of the group consisting of ethylenediamine, ethanolamine, triethanolamine and alcohol.

5. The method of preventing or removing

opalescence in a photographic element which comprises treating the photographic element bearing a polyvinyl resin layer containing a developed and fixed silver image with a solution containing a member of the group consisting of ethylenediamine, ethanolamine, triethanolamine and alcohol.

6. The method of preventing or removing opalescence in a photographic element which comprises treating the photographic element bearing a polyvinyl acetal layer containing a developed and fixed silver image with a solution containing a member of the group consisting of ethylenediamine, ethanolamine, triethanolamine and alcohol.

JOHN I. CRABTREE.  
GEORGE T. EATON.